

1

2,830,868

METHOD FOR RESTORING WHITENESS TO  
YELLOWED NYLON FABRICS

Larry J. Barton, San Leandro, Calif., assignor, by mesne assignments, to The Clorox Company, Cincinnati, Ohio, a corporation of Ohio

No Drawing. Application September 27, 1955  
Serial No. 537,068

6 Claims. (Cl. 8—108)

One of the problems that has arisen over the past few years has been that of white nylon fabrics "age yellowing" to the point that they become unsightly in appearance. The use of white nylon for nurses' uniforms, waitresses' garments, professional people's jackets and similar types—including shirts, underwear and stockings—has widely increased in popularity. These types of articles, if for nothing but appearance, should be maintained in a white and sanitary appearing condition.

The "age yellowing" is the result of a combination of conditions such as exposure of these garments to the atmosphere in general, to the action of sunlight and particularly due to washing effects generally caused by the modern-day type of detergents. As time passes, the yellowing increases in amount to the point where eventually such yellow approaches a light brown in color. It is quite evident that during this yellowing period, such garments become unsightly and are not fit to be used for the purposes for which they are intended.

A great deal of experimental work has been performed to devise some method to eliminate such yellow color and to bring back the fabric to its original whiteness. Substances such as potassium permanganate, hydrogen peroxide, sodium and other alkali metal hypochlorites, sodium sulfite, sodium bisulfite, sulfuric acid and sulfurous acid and sulfonate-formaldehyde salts have been used in an attempt to eliminate this yellow color but with no success.

Various complex treatments have been suggested, such as the use of a detergent to wash the fabric first, followed by the use of a reducing agent and then followed by the use of an oxidizing agent. While such a complex formulation gives fairly good results, it requires a considerable amount of time upon the part of the housewife and requires a combination of operations, such as rinsing between treatments, and does not offer a really satisfactory method of obtaining the end result desired.

One type of product on the market at the present time which aids in the overcoming of such yellow coloring are solutions of optical dyes or Blancophors. These solutions do not remove the yellow, but due to their reflectivity, cover up the yellowing, giving the appearance of renewing whiteness. That this problem is really severe may be ascertained by noting the great number of those optical dye solutions which have appeared on the market during the past year. However, the benefits from the use of such optical dyes are very short-lasting as they are quickly faded by the action of sunlight with the result of a recurring yellowing of the fabric.

Summarizing this invention, it is designed to overcome the foregoing problem, and has as its objects, among others, the provision of a quick, convenient and satisfactory method capable of being readily performed, for example, by any housewife quickly and accurately in her own home, using a composition comprising economical materials which are found in practically every household or which may be quickly obtained at the nearest

2

grocery store, and which will safely restore to their original whiteness "age yellowed" nylon fabrics or garments. Generally, such method comprises treating the nylon with a composition consisting essentially of an aqueous solution of a controlled amount of an hypochlorite bleaching agent together with a controlled amount of an acid, preferably a weak organic acid, such as acetic, citric, malic or tartaric, to impart to the solution critical pH and available chlorine ranges, which will restore the whiteness and yet not damage the nylon.

Such solution will quickly and readily remove the yellow color, bringing the nylon fabric back to its original whiteness and will perform such operation without any undue deterioration to the fabric. For a practical household application, vinegar may be the source of acetic acid, while lemon juice, orange juice or grapefruit juice may be the source of citric acid, and, consequently, may be employed for such purpose. Sodium hypochlorite, in the form of a 5.25% by weight aqueous solution is widely available and is consequently preferred as the bleaching agent in providing the available chlorine in the composition.

In greater detail, numerous experiments made pursuant to this invention establish that the solution is quite critical as to its concentration of available chlorine and as to its pH (a measure of hydrogen ion concentration). To 1.0 gallon of water, optimum results are obtained after adding 2.0 full tablespoons (one ounce) of a 5.25% by weight aqueous sodium hypochlorite solution, together with 1.0 full teaspoon ( $\frac{1}{6}$  ounce) of household vinegar obtained in any grocery store, or lemon juice, orange juice or grapefruit juice. The vinegar and citrus fruit juices contain approximately 5.0% by weight of the weak organic acid. The resultant solution will contain approximately 400 parts by weight per million of available chlorine and will have a pH ranging from approximately 8.00 to 8.30. A solution of approximately 400 parts by weight per million available chlorine made from a sodium hypochlorite solution and water alone would have a pH of approximately 9.30 to 9.70.

The vinegar or citric acid containing fruit juices may vary in the solution of 1.0 gallon of water and 2.0 tablespoonsfuls of the 5.25% sodium hypochlorite solution, from as low as  $\frac{1}{2}$  teaspoonful, which will impart a pH range of approximately 8.50 to 8.70, to as high as 2.0 tablespoonsfuls which will impart a pH ranging from 7.70 to 7.90. Such solutions at a temperature of approximately 125° F., which is the approximate temperature of household warm washing water, will generally remove even the most intense yellow from white nylon immersed therein in 15 to 30 minutes. Even if it should be necessary to repeat such treatment, the fabric will not be adversely affected in tensile strength.

Based upon extensive experimentation, it has been determined that the lowering of the amount of the 5.25% sodium hypochlorite solution, for instance to much below 1.0 tablespoonful per gallon of water with the preferred amount of acid, does not give any better whiteness, but does have a deleterious effect upon the strength of the fabric itself. This is believed so because too little of the hypochlorite results in too low a pH which causes degradation of the nylon. It also has been determined from such experimentation that if the amount of the 5.25% sodium hypochlorite solution is increased to much over 4.0 tablespoonsfuls with the same preferred amount of acid, no better whitening is obtained; and there is a decided weakening of the fabric strength which is believed due to too high a pH. If more of the acid is added, which has the effect of lowering the pH, again there is no increase in whitening capabilities, but

it results in very serious weakening of the nylon fibre itself.

Thus, as a result of the aforementioned experiments, it has been determined empirically that there is a delicate balance between the pH and available chlorine ranges of the solution. At too high or too low a pH, damage or degradation of the fabric results. If the available chlorine content is too low, satisfactory whitening is not obtained while if the available chlorine content is too high, damage to the fibre results. The available chlorine content of the solution should, therefore, not be much below 200 parts by weight per million and should not substantially exceed 800 parts by weight per million, while the pH range should not vary too much from between 7.70 and 8.70 with the optimum results, as aforementioned, of 400 parts by weight per million available chlorine with a pH ranging between 8.00 and 8.30. Any proportions of the acid, hypochlorite and water may be employed to provide these ranges, depending on the concentrations of the acid and the hypochlorite employed, and also the volume of water, as it is immaterial what such concentrations or volume may be.

In this connection, other acids such as boric, oxalic, phosphoric, hydrochloric, nitric or sulfuric could be used under very carefully controlled conditions to provide the pH range indicated, but it is preferred to employ weak organic acids because the amount added to the nylon treating solution need not be so precisely controlled for providing the proper pH range, rendering their use more suitable by non-technical persons in a household. Of such weak organic acids, acetic and citric acid are most desirable because they are present, respectively, in vinegar and citrus fruit juice usually found in the ordinary household.

While an initial aqueous solution of 5.25% by weight sodium hypochlorite is preferred due to its ready availability in any grocery store, calcium hypochlorite, potassium hypochlorite, lithium hypochlorite or any of the organic powdered compounds can be utilized containing a chlorine radical which in the presence of an aqueous solution will develop available chlorine, so long as such nylon treating solution meets the required parts per million of available chlorine, together with the requirements covered by the pH range as described. Also, as previously mentioned, instead of vinegar or the citric acid containing fruit juices, the weak organic acids themselves or other acids can be employed.

The actual treatment of the nylon fabric, which may be any of the fabrics available in stores in the form of garments or otherwise and varying from fine spun fabrics to woven wear, is quite simple. All that need be done is to soak the yellowed fabric in the treating solution for a suitable period of time which may vary from 15 to 40 minutes, depending on the extent of the yellowing and the temperature of the water, then remove the fabric and thoroughly rinse it in clean clear water, preferably at room temperature but which may be warm if so desired. Warm water is preferred for the treating solution; the usual temperature of such water in household washing operations being approximately 125° F., and such temperature is preferred. The soaking should not exceed much over 40 minutes because too long a soaking at one time may weaken the fabric.

No rubbing of the nylon in the treating solution is necessary. The minimum time for the length of soaking is not critical because it is only necessary to allow the nylon to stand immersed for a period sufficient to remove the yellowing, but not long enough to cause damage to the fabric; and if the nylon has been soaked for a time insufficient to remove the yellow, it can be treated again. A minimum of 15 minutes of soaking is desirable, however, and will in no instance cause damage to the fabric.

Warm water is desirable rather than cold or room

temperature water because the action is slightly slower with cold water. However, room temperature or cold water can be employed. Real hot water in the order of 180° to 200° F. or boiling water may be utilized, but is not recommended because although whitening the fabric more quickly, it may damage the same due to the heat alone. In certain cases where the fabric has become highly yellowed, it may be necessary to repeat the treatment of the fabric.

10 After the solution is prepared for the treatment of the nylon, it should be employed relatively promptly, namely, within approximately 24 hours. This is so because the incorporation of the acid results in relatively rapid loss of available chlorine content; and the solution will not hold its available chlorine content for much over 24 hours. Therefore, after preparation, the solution should be used promptly within an hour or two for best results; the sooner the better.

After the nylon has been treated, it will be restored to 20 original whiteness, and will remain white for a period comparable to that of new nylon fabric before the treatment, namely, for about 3 to 4 months. Upon yellowing of the fabric again during usage after a treatment, the 25 original whiteness can again be restored by further treatment with the solution.

The following example is illustrative of the preferred method and composition of the invention:

To 1.0 gallon of clean clear water in the neighborhood of 125° F., add 2.0 tablespoonsful (one ounce) of a 30 5.25% by weight sodium hypochlorite solution, such as is commonly sold as a household bleach and disinfectant in grocery stores, and 1.0 teaspoonful ( $\frac{1}{6}$  ounce) of household vinegar, such household vinegar being standard and containing approximately 5.0% by weight acetic acid. 35 This solution is thoroughly mixed; and promptly after the mixing, the yellowed nylon fabric is immersed and allowed to soak or stand in the solution 15 minutes if only mildly yellowed, and 30 minutes if quite yellowed. At the end of such time, the fabric is separated from the 40 solution by removal therefrom, and thoroughly rinsed clean of the solution in clean clear water at room temperature. The yellowing will in most instances be completely removed without any damage to the fabric. However, in certain instances where a high degree of yellow 45 had occurred, it might be necessary to repeat this operation.

I claim:

1. The method of restoring to whiteness age yellowed 50 nylon garment fabric which consists essentially in the single whitening step of soaking such fabric for a period of about 15 to 40 minutes in an aqueous solution consisting essentially of an hypochlorite and a weak organic acid of the group consisting of acetic acid and citric acid contained, respectively, in household vinegar and citrus fruit juice, said acid being in an amount to provide a pH of said 55 solution ranging from 7.70 to 8.70 and an available chlorine content of from 200 to 800 parts per million, and after such whitening step effecting separation between the garment and said solution.

2. The method of restoring to whiteness age yellowed 60 nylon fabric, which consists essentially of soaking the same for a period of from about 15 to 40 minutes in an aqueous solution consisting essentially of an hypochlorite and a weak organic acid, said solution having a pH ranging from 7.70 to 8.70 and an available chlorine content of from 200 to 800 parts per million, and after such period rinsing the solution from the fabric.

3. The method of claim 2, in which the hypochlorite 65 is sodium hypochlorite, and the acid is of the group consisting of acetic and citric acid contained, respectively, in household vinegar and citrus fruit juice.

4. The method of claim 2, in which the hypochlorite 70 is sodium hypochlorite in an amount which normally provides an available chlorine content of 400 parts per million

and a pH between 9.30 and 9.70 in water solution, and in which the acid is of the group consisting of acetic acid and citric acid, said acid being present in an amount in relation to the amount of hypochlorite to impart a pH of between 8.00 and 8.30 to said solution containing said available chlorine content.

5. The method of claim 2, wherein said hypochlorite is a 5.25% by weight sodium hypochlorite solution present in the proportion of 1.0 to 4.0 tablespoonfuls of said solution per 1.0 gallon of water, and wherein said acid consists of an organic acid of the group consisting of acetic and citric acid contained, respectively, in  $\frac{1}{2}$  to 2 teaspoonfuls of household vinegar and citrus fruit juice per gallon of water.

5

10

6. The method of claim 1 in which the amount of said sodium hypochlorite solution is 2.0 tablespoonfuls, and the amount of said acid is 1.0 teaspoonful.

**References Cited in the file of this patent**

**UNITED STATES PATENTS**

|           |                 |               |
|-----------|-----------------|---------------|
| 2,105,839 | McNutt          | Jan. 18, 1938 |
| 2,113,453 | Mitchell et al. | Apr. 5, 1938  |
| 2,727,804 | Lutgerhorst     | Dec. 20, 1955 |

**OTHER REFERENCES**

Ridge et al.: J. Textile Institute, May 1942, pages 162-164.

U. S. DEPARTMENT OF COMMERCE  
PATENT OFFICE

CERTIFICATE OF CORRECTION

Patent No. 2,830,868      Larry J. Barton

April 15, 1958

It is hereby certified that error appears in the printed specification of the above numbered patent requiring correction and that the said Letters Patent should read as corrected below.

Column 6, line 1, for the claim reference numeral "1" read -- 5 --.

Signed and sealed this 17th day of June 1958.

(SEAL)

Attest:

KARL H. AXLINE

Attesting Officer

ROBERT C. WATSON  
Commissioner of Patents